

## UNITED STATES PATENT OFFICE

2,250,545

## LUBRICATING COMPOSITION

Louis A. Mikeska, Westfield, and Eugene Lieber,  
Linden, N. J., assignors to Standard Oil Development Company, a corporation of Delaware

No Drawing. Application October 19, 1938,  
Serial No. 235,778

8 Claims. (Cl. 252—46)

This invention deals with lubricating compositions. More specifically, it relates to the use in such compositions of small amounts of soluble organic xanthogen tetrasulfides which are believed to possess a structure corresponding to the following formula:



where R and R' represent alkyl, cyclic, or cyclo-alkyl organic groups.

These compounds are condensation products which may be obtained in high yields according to the following reactions:



An example in the preparation of such a material (ethyl xanthogen tetrasulfide) is as follows:

Potassium hydroxide is dissolved in absolute alcohol (fair excess over that required for reaction) and the required amount of carbon disulfide is added with cooling and mechanical agitation. Potassium xanthate precipitates out. The amount of xanthate is further increased by the addition of ether. (In large production, the excess alcohol being saturated with xanthate could be used again, avoiding the use of ether as a precipitant.) The solid product is recovered by filtration and dried.

The potassium xanthate is suspended in benzene (other inert solvents such as light naphtha could be used), stirred and a benzene solution of sulfur monochloride added with cooling. After the sulfur chloride has been added, the reaction mixture is refluxed for 2 hours to complete the condensation, and then poured into water. The benzene layer is removed and dried. After stripping off the benzene, the xanthogen tetrasulfide remains as a residue.

The overall yield averages around 86.7%.

These xanthogen tetrasulfides possess such unusual characteristics as to impart to lubricating and other oils, new and unexpected properties. For example, they possess excellent antioxidant

and corrosion inhibiting properties. They likewise exhibit exceptionally potent extreme pressure lubricating properties. Although they are sulfur compounds (ethyl xanthogen tetrasulfide contains about 63% S), they are light colored, oil soluble compounds, possessing a faint pleasant odor, and thus impart no objectionable characteristics to the mineral or other oil base stock in which they are blended. These compounds are also compatible with soap, fatty oils and other ingredients normally employed in soluble oils, cutting oils, greases, motor oils, compounded, and industrial lubricants, without causing precipitation or settling out of sulfur or sulfur compounds.

In the extreme pressure lubricating art the common practice is to add to the lubricating oil a sulfurized mineral or fatty oil. These compounds are generally dark colored, odorous materials, poor in combined sulfur. Alkyl sulfides and polysulfides have been proposed for this purpose but their pungent and sickening odor markedly limits their uses in this direction. Xanthogen disulfides, prepared by the oxidation of xanthic salts show relatively poor load carrying properties, a 5% blend failing on the S. A. E. machine at 200 lbs. load. Although ethyl xanthogen trisulfide shows fair load carrying properties, it tends to settle out free sulfur on standing, and is therefore excluded from use to some extent because of its instability. An improved composition can be obtained by chilling the trisulfide or its solutions and filtering to remove the separated material.

However, the xanthogen tetrasulfides (e. g. ethyl xanthogen tetrasulfide), such as those embodied in the present invention, give excellent results as extreme pressure blending agents. When used alone in mineral lubricating oil, 3% of this material will carry the full load (580 lbs.) on the S. A. E. machine at 1000 R. P. M., and in addition, it meets the requirements of the Packard Stability Test. This test involves the heating of the blend in an oven at 200° F. for 64 hrs. and running the thus-treated oil on the S. A. E. machine at 1000 R. P. M. and 83.6 lbs./sec. loading rate, the rubbing ratio being 14.6:1. The blend must carry a full load of 550 lbs. scale pull.

Blends containing these xanthogen tetrasulfides have shown no sulfur separation at 0° F. for periods of over 20 days.

In the condensation reaction, it is possible to employ sulfur dichloride, rather than sulfur monochloride, as well as phosphorus halides. The best results, however, are obtained with sul-

fur monochloride. The alkyl, aryl, or aralkyl groups (R and R') may be methyl, ethyl, propyl, amyl, lauryl, oleyl, benzyl, dibenzyl, phenyl ethyl, phenyl, naphthyl, diphenyl, naphthene, cyclohexyl, and the like. Two different groups may be present in the molecule when a mixture of xanthate salts is condensed. It is also possible to replace the oxygen atoms present in the molecule by sulfur, by employing mercaptans instead of the alcohol for the preparation of the xanthate salt prior to condensation. Since these products pick up some of the mercaptan odor which is difficult to remove, they are not as desirable as the corresponding alcohol derivatives.

One exceptionally wide use for the compositions which are the subject of this invention, is in the field of cutting oils. Here a high E. P. effect is desired without any detrimental odor or discoloration of the base stock, so as to give clean work pieces without need for further handling or processing. For this purpose, it is desired to employ about 2 to 10% of the tetrasulfide condensation products previously described. Soluble cutting oils are prepared by the addition of emulsifiers such as sodium naphthenate, mahogany soaps, rosin soaps, glycerol, alcohol and similar ingredients. The lubricating oil base stocks are generally crude or refined mineral oils of about 70 viscosity at 100° F. (Saybolt) to about 5000 viscosity at 100° F.

In many cases, where antioxidant and anti-corrosion effects are more desired, about 0.01 to 2% of the xanthate tetrasulfides is sufficient. For the preparation of E. P. greases and gear oils, higher viscosity base stocks may be employed, and there is often an advantage to employ stocks of high viscosity index, e. g. above 50.

The present compositions may be employed in conjunction with linear polymer V. I. improvers, pour inhibitors, dyes, resins, voltolized fats and/or mineral oils or waxes, ester and other oiliness agents, phenolic or amino oxidation inhibitors, soaps, such as calcium stearate, lead oleate, lead naphthenate, aluminum naphthenate, and the like, dyes, halogenated compounds, such as chlorinated esters, chlorinated paraffin waxes, etc., wetting agents, insecticides, germicides, fungicides, and the like.

The invention is not limited to any theory of structure or action, but is limited only by the claims in which it is the intention to cover the invention as broadly as the prior art permits.

We claim:

1. A lubricating composition comprising a mineral lubricating oil and 0.01 to 10% of a soluble organic xanthogen tetrasulfide.

2. A lubricating composition according to claim

1 in which the tetrasulfide is an alkyl xanthogen tetrasulfide.

3. A lubricating composition according to claim 1 in which the tetrasulfide is ethyl xanthyl tetrasulfide.

4. A lubricating composition according to claim 1 in which the mineral oil is an oil of high viscosity index.

5. A cutting oil comprising a mineral lubricating oil and about 2 to 8% of a soluble xanthogen tetrasulfide having the probable structure:



15 where R and R' are alkyl, cyclic or cyclo-alkyl groups, and the oxygen atoms may be replaced by sulfur.

6. A composition of matter comprising an oil selected from the group consisting of mineral oils and fatty oils, and a small amount of organic xanthogen tetrasulfide.

7. A lubricating composition comprising a lubricating oil base stock and at least about .01% of a soluble xanthogen sulfide having the general formula:



30 where R and R' are like or unlike alkyl, cyclic hydrocarbon, or mixed cyclo-alkyl radicals, and X is either oxygen or sulfur.

8. The method of preparing improved lubricating compositions which comprises reacting a compound having the general formula  $\text{R}-\text{X}-\text{H}$  where R is an alkyl, cyclic hydrocarbon, or mixed cyclo-alkyl radical and X is either oxygen or sulfur, with carbon disulfide and with a metal hydroxide to form a xanthate having the general formula:



35 where M represents the metal, then reacting 2 mols of such xanthate in which the R constituents are like or unlike, with sulfur monochloride in the presence of an inert hydrocarbon solvent, refluxing the mixture to complete the condensation, contacting the reaction mass with water to dissolve the metal chloride formed as by-product, separating the reaction mass into an organic solvent layer and an aqueous layer, removing the aqueous layer, removing the solvent from the solvent layer to obtain the organic condensation product as a residue, and dissolving a small amount of said residue in a lubricating oil base stock.

LOUIS A. MIKESKA.  
EUGENE LIEBER.

## DISCLAIMER

2,250,545.—*Louis A. Mikeska, Westfield, and Eugene Lieber, Linden, N. J. LUBRICATING COMPOSITION. Patent dated July 29, 1941. Disclaimer filed April 14, 1942, by the assignee, Standard Oil Development Company.*

Hereby enters this disclaimer to claims 1, 2, 3, 6, and 7.

[Official Gazette June 2, 1942.]